

Feb. 9, 1932.

S. P. MILLER

1,844,900

HIGH CARBON PITCH COMPOSITIONS

Filed Dec. 29, 1927

3 Sheets-Sheet 1



INVENTOR  
Stuart Pardee Miller  
BY  
Pennie Davis, Marvin, Edwards  
ATTORNEYS

Feb. 9, 1932.

S. P. MILLER

1,844,900

HIGH CARBON PITCH COMPOSITIONS

Filed Dec. 29, 1927

3 Sheets-Sheet 2



INVENTOR  
S. P. MILLER  
BY  
Dennis, Davis, Marvin, & Edwards  
ATTORNEYS

Feb. 9, 1932.

S. P. MILLER

1,844,900

HIGH CARBON PITCH COMPOSITIONS

Filed Dec. 29, 1927

3 Sheets-Sheet 3



INVENTOR

*Stuart Parmelee Miller*  
BY  
*Pennie, Davis, Marion & Edmunds*  
ATTORNEYS

## UNITED STATES PATENT OFFICE

STUART PARMELEE MILLER, OF ENGLEWOOD, NEW JERSEY, ASSIGNEE TO THE BARRETT COMPANY, OF NEW YORK, N. Y., A CORPORATION OF NEW JERSEY

## HIGH CARBON PITCH COMPOSITIONS

Application filed December 29, 1927. Serial No. 243,308.

This invention relates to new pitch compositions. The invention relates particularly to pitch compositions of regulated high carbon content.

5 In the ordinary operation of by-product coke oven and gas retort plants, the coal distillation gases are cooled to separate tar therefrom and the tar is shipped to tar distillation plants for distillation. The pitches 10 produced from ordinary coke oven tar have too low a free carbon content to make them available for certain purposes. Pitches containing a high free carbon content are obtained ordinarily from the distillation of 15 gas retort tars, particularly horizontal gas retort tars, or the admixture of such tars with coke oven tar and the distillation of the mixture. So also, pitches produced from gas retort tars alone may not have the proper 20 carbon content and other properties.

According to the present invention, the gases given off from the coke ovens or gas retorts near the end of the coking or gas making period are kept separate and cooled for 25 the separation therefrom of a relatively high carbon tar, which tar is subjected to distillation for the production therefrom of a high carbon pitch, and the resulting high carbon pitch is blended with tar or a low melting 30 point pitch to produce the new pitch compositions.

In referring to carbon and free carbon in the tar and pitch, I use these terms in their ordinary meaning to include not only elemental or molecular carbon but also those constituents which remain as insoluble residue on digestion of the tar or pitch with benzol or similar solvent. It may include certain inorganic impurities as well as insoluble hydrocarbons of high molecular weight.

In my companion application, Serial No 35 243,307 I have described the production of new high carbon pitches at coke oven or other coal distillation plants by separately collecting the gases from near the end of the coking period, cooling the gases to separate high carbon tar therefrom, and distilling the high carbon tar to produce new high carbon 40 pitches. The present invention produces new

products of a composite and somewhat different character. The new high carbon pitches produced in accordance with said companion application can advantageously be employed according to the present invention in producing the new composite pitch 55 products.

In my companion application, Serial No. 243,305 I have described the production of low carbon pitches by separately collecting 60 the gases from the early period of the coking operation, cooling the gases to separate a low carbon tar therefrom, and distilling such tar to produce low carbon pitches; and in my companion application, Serial No. 243,306. 65 I have described the blending of such pitches with tar to give new composite pitch products. The production of the new products of such applications, can if desired, be combined with the production of the products of 70 the present invention; although the present invention is not limited to operations in which it is so combined with the processes and the production of the products of such companion applications. 75

In the practice of the present invention, I provide for the separate collecting of the coke oven or other coal distillation gases given off during the later portion of the coking operation, when the gases are lower in 80 tar content, and when the tar content of the gases is a higher carbon tar than during the earlier period of the coking operation. These gases with their high carbon content are cooled to separate therefrom a high carbon tar, 85 which tar is subjected to distillation for the production therefrom of a high carbon pitch. These operations can be carried out in accordance with the process and to produce the product described in my companion application, Serial No. 243,307 but the distillation of the tar will be carried to such a point that a relatively high melting point pitch will be produced of high carbon content, which pitch I then blend with additional tar or lower melting point pitch to produce new composite 90 products. 95

The present invention is of particular value for the production of high carbon pitch products of relatively low melting point and of 100

higher carbon content than can be obtained by the ordinary distillation of coal tar. For example, for certain purposes such as road-making purposes, relatively low melting point pitches are required having a melting point around 105 to 110° F. and containing a carbon content around 12 to 15%. Such pitches ordinarily require the addition of high carbon gas retort tar to coke oven tar before distillation. Such pitches can readily be produced according to the present invention by subjecting the high carbon tar from the coke oven gases to distillation to produce a high carbon pitch of high melting point and then blending this pitch in proper proportion with tar or soft pitch, either without or with further distillation of the mixture to remove additional oils therefrom. For example, the high carbon pitches can be produced of melting point around 145 to 165° F., or even around 225 or 250 or even 300° F., or higher, and such high carbon pitches can then be blended with tar or soft pitch to produce the new composite products.

25 The distillation of the high carbon tar and the production of the high carbon pitch which is to be blended with the additional tar or soft pitch is advantageously carried out at the coke oven or gas retort plant by bringing the tar into direct and intimate contact with the hot coal distillation gases; and this operation can be carried out in a continuous manner, with the continuous production of the high carbon pitch, and the continuous blending of such pitch with the tar or soft pitch to produce the new composite products in a continuous manner.

In the production of the new product at coal distillation plants, for example, at coke oven plants, I provide a plurality of collector mains, one for the gases from near the end of the coking operation from which the high carbon tar is to be separated, and another for the gases from the earlier period of the coking operation from which a lower carbon tar is separated; and I provide in addition separate condensing systems for the further condensation of light tar or tarry oil from the respective gases. The heavy tars from the collector mains and the lighter tars or tarry oils from the condensers are kept separate. The high carbon tars from the collector main and condensers may be combined together for distillation or distilled separately. Similarly, the lower carbon tars from the collector main and condensers may, if desired, be subjected to distillation either in admixture or separately to produce low carbon pitches, although such low carbon tars can be utilized for other purposes.

60 In addition to such separate condensing and collecting systems and apparatus for keeping separate the respective tars, I provide a distillation apparatus for distilling the high carbon tar or tars together or separately, which

distillation apparatus is advantageously one in which the distillation is effected by direct and intimate contact with hot coal distillation gases. This can be carried out in various ways, such as by the provision of a still or short collector main into which the tar to be distilled is introduced and into which the gases from a selected number of ovens are introduced at a high temperature, and in which the tar is brought into intimate contact with the hot gases, as by spraying or atomizing the tar into the gases by means of spray nozzles or mechanical agitating devices such as rotary discs or rotary rolls, etc., rotating at a high rate of speed to atomize the tar and bring it into intimate contact with all parts of the gas in the still. By introducing the high carbon tar continuously and withdrawing the high carbon pitch continuously, the high carbon pitch is available in a highly heated state for blending with the tar or soft pitch and this blending can advantageously be carried out with utilization of the heat of the hot pitch for assisting in the blending operations and for heating and in some cases if desired, for distilling the lighter oils from the tar blended therewith.

The character and particularly the melting point of the pitch produced may be varied by varying the extent to which the distillation is carried, but the distillation will in most cases be carried sufficiently to produce a pitch of relatively high melting point, as compared with the melting point of the desired pitch composition. The maximum melting point will in some cases be limited by the free carbon content of the pitch, since a very high carbon content pitch is in general more difficult to handle and to circulate and to keep fluid than a pitch of lower free carbon content but of corresponding melting point. In general, however, the melting point of the high carbon pitch produced will be determined by the desired character of the pitch composition resulting from the blending of the high carbon pitch with tar or with a lower melting point pitch. For example, a pitch of a melting point of about 105 to 110° F., to be used for road construction can be made by blending pitch of not higher than 165° F. melting point with the required amount of tar to reduce the melting point to 105 to 110° F. However, it is readily possible to produce high carbon pitches of melting points up to 300° F. and in some cases up to 400° F. or higher. Such distillation gives a high yield of oils of high specific gravity and some of them of high boiling point. Some increase in carbon content may take place during the distillation of the high carbon tar by means of the hot coke oven gases, but this increase will be much less than when the high carbon tars are distilled in ordinary externally heated tar stills. The carbon content of the pitch can be regulated and controlled to a greater

or less extent by selecting the period of operation of the coke ovens during which the gases are collected for the separation of tar therefrom, thereby recovering tars of higher or less high carbon content, from which pitches of somewhat varying high carbon content can be produced.

The tar which is blended with the high carbon pitch, according to the present invention, 10 may be varied in accordance with the character of the composite pitch desired. For some purposes, the tar to be blended with the high carbon pitch may itself be high carbon tar such as is separated from the lean gases near 15 the end of the coking operation. Blends of such tars with the high melting point and high carbon pitches will give composite pitch products of intermediate melting point but of relatively high carbon content. For some 20 purposes, a much lower carbon content of the blended mixture is sufficient, and, in such cases, the tar blended with the high carbon pitch may be ordinary coke oven tar with its normal carbon content, that is, coke oven tar 25 such as is obtained when the total tar from the various ovens is collected together. In some cases, the low carbon tars produced from the rich gases given off during the early period of the coking operation may be blended to a 30 greater or less extent to regulate and control the carbon content of the blended product.

The separate collection of high and low carbon tars at the coke oven plant and the separate distillation of the high carbon tar 35 to produce high carbon pitch gives various products at the coke oven plant for blending in an undistilled condition with the high carbon pitch. For example, the heavy tar from the collector main in which the high carbon 40 tar is collected, may be employed for blending purposes, and its relatively lower oil content makes it particularly valuable for that purpose. So also, where ordinary heavy tar from the collector main in which all of the 45 tar from the ovens is collected together, is available, this may be blended with the high carbon pitch to form new composite products. The tar which is blended with the high carbon pitch may itself be subjected to an initial or partial distillation to dehydrate it or to 50 free it from lower boiling oils, although in some cases the raw tar may be employed without such distillation or dehydration. By regulating the amount of the tar and pitch blended 55 with each other and the carbon content of the pitch and the tar, composite products of intermediate carbon content and melting point can be produced, and this can be regulated by regulating and controlling the character of the individual products which are 60 blended with each other. I do not, however, exclude the blending of tars other than coke oven tars with the new high carbon pitches, since in some cases tar from other sources, 65 such as gas-house tars, may be employed.

The products of the blending of different tars, etc., with the high melting point high carbon pitches, will differ in characteristics, depending upon the nature of the materials employed.

The blending of the high melting point pitch with tar is accomplished preferably by introducing continuous streams of the hot thinly fluid materials to be blended into a suitable receptacle, the streams being directed 75 so that they flow together and thus immediately produce a uniform blended product. Such operation is particularly desirable if the tar which is introduced contains water because the temperature of the pitch may be 80 such as to vaporize the water immediately together with some of the more volatile constituents of the tar, thus producing a dehydrated product. The vaporized water and oil constituents can be withdrawn continuously 85 from the receptacle and the oil can be condensed by the provision of a suitable condenser. The oil can, after separation of water, be returned to the pitch, if desired. The blended product can likewise be withdrawn 90 continuously from the receptacle and delivered to suitable storage containers.

As an example of the practice of the invention the gases from the latter portion of the coking period of a coke oven plant can be 95 cooled in the separate collector main by ammonia liquor or ammonia liquor and tar supplied thereto and the separated heavy tar containing a relatively high free carbon content can be distilled then in a separate distillation main by contact with the hot gases from the ovens to produce a pitch having a melting point of, for example, from 165° to 225° F. or up to 300° F. or higher. To produce a road-treating pitch having a melting 100 point of approximately 105° F. and a free carbon content of around 12 to 15%, the desired high melting point pitch can be blended continuously in the manner described with a suitable proportion of raw tar from the same 105 plant from other coke oven batteries or with tar from gas retorts or similar coal distillation plants. The proportion of tar thus blended with the high melting point pitch will depend upon the particular characteristics of the material employed. The amount can be determined readily by test and the blending can be so conducted as to produce a uniform road-treating pitch having the desired melting point with the proper 110 proportion of free carbon.

In applying the invention at gas retort plants, or with gas retort tars, it is possible to produce new composite pitch products varying with the particular tar employed. 115 Horizontal and inclined gas retort plants, which give high carbon tars, will give unusually high carbon tars from the gases given off during the latter part of the gas making operation, and these tars on distillation will 120 130

give high carbon pitches which can be blended with additional tar of the same kind to give unusually high carbon blended products, or with lower carbon tars to give lower carbon pitch compositions. The high carbon tars from the later part of the operation of intermittent vertical retorts will on distillation give pitches of higher carbon content than those obtained from the total tar produced at such plants, but it may be much lower than that obtained at horizontal retort plants, or even at coke oven plants. By blending these various high carbon pitches with tars of varying kinds a wide range of composite blended products can be produced.

The invention may be applied to existing coke oven plants or to gas retort plants, without any considerable modification thereof except for the provision of the separate collector mains, separate tar collecting receptacles and the distillation and blending apparatus. The operation as described permits the recovery of valuable products which have not been available heretofore as the result of coke oven or gas retort operation.

The production of the new compositions will be further described in connection with the accompanying drawings, in which—

Fig. 1 is a plan view of a portion of a coke oven battery;

Fig. 2 is a cross-sectional view of one of the collector mains;

Figs. 3 and 4 are enlarged sectional views of the short collector main; and

Figs. 5 and 6 are details in section of the blending apparatus.

Referring to the drawings, 5 indicates a battery of ovens which are connected by uptake pipes and goose-necks 6 to valve boxes 7 which communicate with collector mains 8 and 9. Valves 10 are arranged in the valve boxes to permit the direction of the hot coke oven gases into one or the other of the collector mains, depending upon the stage of the coal distillation operation in the particular oven to which the valve box is connected. Thus, by operating the valves "rich" and "lean" gases from the several ovens of the battery can be collected separately in the collector mains wherein they are cooled to the desired extent by ammonia liquor introduced through spray nozzles 11 which are supplied through a pump 12 and pipe 13 from a source of ammonia liquor such as a tank 15.

From the collector mains the gases carrying oil vapors and partially condensed tarry constituents are delivered through cross-over mains 16 and 17 to condensers 18 and 19 in which the gases are further cooled to separate the tarry oil constituents. The oil, together with ammonia liquor, can be withdrawn through pipes 20 and 21 and delivered to decanters 22 and 23 wherein the ammonia liquor is separated from the tarry oil. The tarry oil can be delivered to suitable storage

receptacles and the ammonia liquor can be returned if desired for further use as a cooling medium either in the collector mains or in the condensers. The gases escaping from the condensers are delivered through pipes 24 and 25 to exhausters 26 and 26' and thence to equipment (not shown) for the separation of ammonia, light oils, etc.

The tar which separates in the collector mains can be withdrawn through pipes 27 and 28 to decanters 29 and 30, in which ammonia liquor is separated while the tar is stored in tanks. The ammonia liquor may be returned to the collector mains for cooling or may be utilized to recover ammonia therefrom.

The tar from the "lean" gas main contains a relatively high proportion of free carbon and this tar is subjected to distillation in a suitable still such, for example, as a short collector main or still 31 which is disposed preferably at the rear of the ovens and is connected to a plurality of ovens so that hot coal distillation gases pass continuously through the short collector main or still. The tar to be distilled may be introduced to the short collector main or still at one end through pipe 32 by pump 33. The collector main or still 31 is filled with a cylinder 34 adapted to be rotated at a high rate of speed by electric motor 35. The cylinder dips into

the body of tar and pitch in the bottom of collector main or still 31 and atomizes the tar and pitch, in the form of a finely disseminated spray, into the gases passing through the collector main or still 31. The gases are thus effectively scrubbed by the tar and pitch.

In thus mingling with the hot gases the tar is distilled to produce pitch which is withdrawn continuously at 36 and the volatile constituents are separated and join the gases which run through settling tower 46 in which the tar spray and globules and other entrained matter settle out of the scrubbed gases and are returned to the collector main or still 31. The tower 46 may if desired contain baffles or packing. The gases may be withdrawn continuously through a pipe 37 and delivered to a condenser 38 located at any suitable place, wherein the oil constituents can be separated from the gases. Thereafter the gases may be delivered through a pipe 39 to an exhauster and mingled with the remaining gases from the ovens of the battery.

The pitch produced is withdrawn continuously at 36 into receiver 47 from which it is conveyed by pipe 40 and delivered to the blending apparatus 41 comprising a chamber into which the pitch, still at high temperature, is introduced. The tar or other material to be blended with the pitch is similarly introduced through a pipe 42, the two pipes being directed so that the streams are mingled as they enter the chamber as shown in Fig. 6. The tar and pitch thus intimately mingle and

blend to produce a product having the desired characteristics which can be withdrawn continuously through a pipe 43 and delivered to suitable storage receptacles or the blended materials may be withdrawn batchwise.

Owing to the relatively high temperature of the pitch the tar which is blended therewith will be heated and any small amount of moisture present therein together with some lighter oil constituents will be vaporized immediately upon contact between the tar and pitch. The vapor can be withdrawn as it is released through a pipe 44 and delivered to a condenser 45 wherein it is cooled. The oil thus recovered can be mixed with oil obtained by the cooling of other gases from the system, or can be returned to the pitch in 41.

The mixing of the hot high carbon pitch, while at a high temperature, with the tar in the mixing chamber 41, preferably takes place continuously, and any foaming due to heating of coal tar containing water by the hot pitch is readily taken care of. The continuous flow of the tar and the pitch causes the blending of the pitch and tar continuously to give a resulting composite blended product which is still sufficiently hot to be thinly fluid and to run from the apparatus, although the blended product on cooling may be a solid product of higher or lower melting point. The tar which is thus added to and blended with the hot high carbon pitch may itself be preheated and dehydrated or partly distilled to remove part of the light oils therefrom, although such preheating and dehydration may in some cases be omitted and raw wet tar employed. The tar may, as above pointed out, be itself a high carbon tar, or a low carbon tar, or an ordinary normal carbon tar, depending upon the carbon content and other properties of the blended product. The tar need not be a coke oven tar, but may be water gas tar, gas house tar, vertical retort tar, low temperature tar, etc.

This production of the new blended product is carried out at a coke oven plant, with elimination of the transportation of coke oven tar to tar distillation plants or of high carbon gas retort tar to tar distillation plants, and with the production of the new composite product by distilling only a limited amount of high carbon tar which, however, is distilled to give a large yield of oils therefrom of high specific gravity and relatively high boiling point.

The new composite pitch products will be made up of the tar utilized in producing them and of the high carbon pitch blended therewith to form a homogeneous product. These composite products will differ in character from pitches of the same melting point produced by direct distillation of the high carbon tar.

The process of producing the new compo-

site products differs from the process of producing the new high carbon pitches of my companion application, Serial No. 243,307, in that it does not rely upon distillation of all of the tar employed to produce the pitch desired, but subjects only part of the high carbon tar to distillation to produce therefrom a high melting point high carbon pitch and a high yield of distillate oils, including oils of high boiling point, which high melting point pitch is then blended with additional undistilled tar to produce the new composite products. The production of the new compositions involves the distillation of less tar, but distillation to a much higher melting point pitch, as compared with the production of the compositions of said companion application when such pitches are of intermediate melting point.

In its broader aspects, production of the new compositions is not limited to the continuous distillation of the tar to produce the high carbon pitch, nor is it limited to the continuous blending of the hot high carbon pitch as produced with the tar, although the process is advantageously carried out in a continuous manner with continuous distillation of the tar and continuous production of pitch and with continuous blending of the hot high carbon pitch with the raw tar, or with specially treated tar, to produce the new composite pitch products.

While production of the new pitch compositions has been more particularly described in connection with coke oven operation and the production of coke oven tar pitches, it is applicable to other coal distillation plants and tars, such as certain gas retort plants and tars, to produce new composite pitch products.

I claim:—

1. New composite blended pitch compositions, comprising high free carbon pitch of high melting point blended with a substantial amount of coal tar, said coal tar including low boiling constituents not present in a straight distillation pitch of the same melting point as the composite blended pitch composition, the high carbon pitch resulting from the distillation of high carbon tar produced from coke oven or other coal distillation gases during the latter period of the coking of coal in coke ovens or other coal distillation apparatus.

2. New composite blended pitch compositions with a melting point of at least 105° F. and a free carbon content of at least 12%, consisting of a substantial amount of coke oven tar blended with high free carbon pitch of high melting point resulting from the distillation of high carbon coke oven tar recovered from coke oven gases during the latter period of the coking of charges of coal in coke ovens, the coke oven tar comprising

**6**

**1,844,800**

lower boiling constituents not present in a  
pitch produced by the straight distillation  
of the coke oven tar to pitch of the same  
melting point as the composite blended pitch  
composition.

5 In testimony whereof I affix my signature.

STUART PARMELEE MILLER.

**10**

**15**

**20**

**25**

**30**

**35**

**40**

**45**

**50**

**55**

**60**

**65**